



US005359773A

## United States Patent [19]

Nagai

[11] Patent Number: 5,359,773

[45] Date of Patent: Nov. 1, 1994

## [54] MANUFACTURING METHOD OF THE ROLL MAIN BODY OF A CALIBER ROLL

[75] Inventor: Masayuki Nagai, Suita, Japan

[73] Assignee: Sumitomo Metal Industries, Ltd., Osaka, Japan

[21] Appl. No.: 102,952

[22] Filed: Aug. 6, 1993

|           |         |                           |
|-----------|---------|---------------------------|
| 62-109926 | 5/1987  | Japan .                   |
| 63-101012 | 5/1988  | Japan .                   |
| 64-11945  | 1/1989  | Japan .                   |
| 1053708   | 3/1989  | Japan .                   |
| 0307607   | 12/1990 | Japan ..... 72/252.5      |
| 0307608   | 12/1990 | Japan ..... 72/252.5      |
| 4-100615  | 4/1992  | Japan .                   |
| 41-72113  | 6/1992  | Japan .                   |
| 64944     | 3/1971  | Luxembourg .              |
| 555961    | 4/1977  | U.S.S.R. ..... 29/895.212 |
| 1488043   | 6/1989  | U.S.S.R. ..... 72/252.5   |

## Related U.S. Application Data

[62] Division of Ser. No. 833,527, Feb. 11, 1992, abandoned.

## [30] Foreign Application Priority Data

Dec. 5, 1991 [JP] Japan ..... 3-349698

[51] Int. Cl.<sup>5</sup> ..... B23P 11/02

[52] U.S. Cl. ..... 29/895.212; 29/447; 492/34

[58] Field of Search ..... 29/895.212, 895.2, 447; 492/34, 35, 40, 53, 58

## [56] References Cited

## U.S. PATENT DOCUMENTS

|           |         |                  |            |
|-----------|---------|------------------|------------|
| 692,478   | 2/1902  | Robbins et al.   | 29/121.6 X |
| 3,218,691 | 11/1965 | Carroll          | 29/132 X   |
| 3,609,849 | 10/1971 | Krol             | 29/132     |
| 3,793,869 | 2/1974  | Hufnagl et al.   | .          |
| 3,842,471 | 10/1974 | Polhall et al.   | 29/132 X   |
| 4,674,312 | 6/1987  | Cook             | 29/130 X   |
| 4,777,822 | 10/1988 | Uemura et al.    | 72/366.2   |
| 4,817,410 | 4/1989  | Yatsuzuka et al. | 29/130 X   |
| 4,819,471 | 4/1989  | Cook             | 29/132 X   |

## FOREIGN PATENT DOCUMENTS

|           |         |                      |
|-----------|---------|----------------------|
| 54-157757 | 12/1979 | Japan .              |
| 55-28358  | 2/1980  | Japan .              |
| 0070406   | 5/1980  | Japan ..... 72/252.5 |
| 56-86611  | 7/1981  | Japan .              |
| 59-2561   | 1/1984  | Japan .              |
| 1136658   | 6/1986  | Japan ..... 29/132   |
| 61-216807 | 9/1986  | Japan .              |

Primary Examiner—Timothy V. Eley

Attorney, Agent, or Firm—Burns, Doane, Swecker &amp; Mathis

## [57] ABSTRACT

A caliber roll for rolling consisting of a roll main body having a caliber on the outer circumference and provided with a shaft hole penetrating in the axial direction, and a roll shaft inserted into the shaft hole of the roll main body, in which a compressive stress in the widthwise direction of the roll main body is applied to the bottom of the caliber. This compressive stress is applied by forming either the inner circumference of the roll main body or the circumference of the roll shaft in a taper, and shrinkage-fitting or cold-fitting the roll main body and the roll shaft, or by pressing the both end faces in the widthwise direction of the roll main body by means of a pressing jig fixed to the roll shaft. In addition, a recess gap is provided in either one or both of the inner circumference in the middle of the widthwise direction of the roll main body and the corresponding circumference of the roll shaft. The roll main body is composed of an iron-based alloy including, by weight, C: 0.75 to 1.75%, Si: 3.0% or less Mn: 2.0% or less, P: 0.30% or less, S: 0.030% or less, Cr: 5.0 to 13.00%, Mo: 0.80 to 5.0%, and V: 0.1 to 0.5%, in which the entire hardness is adjusted to HRC 52 to 56, and the metal flow is in the axial direction.

9 Claims, 21 Drawing Sheets



Fig. 1  
Prior Art



Fig. 2  
Prior Art



Fig. 3  
Prior Art



Fig. 4



Fig. 5



Fig. 6



Fig. 7(a)



Fig. 7(b)





Fig. 9



Fig. 10



Fig. 11



Fig. 12



Fig. 13



Fig. 14



Fig. 15



Fig. 16



Fig. 17



Fig. 18



Fig. 19



Fig. 20



Fig. 21



## MANUFACTURING METHOD OF THE ROLL MAIN BODY OF A CALIBER ROLL

This application is a divisional of application Ser. No. 5 07/833,527, filed Feb. 11, 1992 now abandoned.

### BACKGROUND OF THE INVENTION

#### 1. Field of the Invention

The present invention relates to a caliber roll for 10 rolling consisting of a roll main body and a roll shaft, used in caliber rolling of tubes and bars, and a manufacturing method of making its roll main body, and more particularly to a caliber roll for rolling possessing a sufficient abrasion resistance and crack resistance characteristic and having an excellent service life, and a manufacturing method of making its roll main body.

#### 2. Description of the Related Art

A caliber roll for rolling used in caliber rolling of tubes and bars has, as shown in FIG. 1, a hollow roll main body 1 having a caliber 1a, and a roll shaft 2 tightly fitted into a shaft hole 1b of the roll main body 1. In the case of this caliber roll for rolling, when rolling, a tensile stress  $\sigma_t$  acts on the bottom section of the caliber 1a of the roll main body 1, due to the surface pressure P acting on the caliber 1a of the roll main body 1. The distribution of this tensile stress  $\sigma_t$  reaches the maximum on the bottom surface of the caliber 1a, and supposing this maximum value to be  $\sigma_{tmax}$ , the surface pressure P is high depending on the rolling condition, and  $\sigma_{tmax}$  rises, and when this  $\sigma_{tmax}$  exceeds the material strength of the roll main body 1, the bottom surface of the caliber 1a is cracked, and thereby the roll main body 1 is broken. Besides, the bottom surface of the caliber 1a of the roll main body 1 is likely to be cracked 35 because it is exposed to cyclic thermal stresses of processing heat and cooling by lubricating oil.

As the countermeasure of roll breakdown, hitherto, the roll material is changed to a stronger material, but the roll cost rises, and generally the higher the strength, the lower becomes the toughness, and cracks due to 40 impact are more likely to occur.

As another method, a gap is provided in the contact surfaces of the roll main body 1 and roll shaft 2 (Japanese Patent Application Publication No. 59-2561, U.S. Pat. No. 4,674,312 (Japanese Patent Application Laid-Open No. 61-216807)). These methods are intended to lessen the tensile stress on the bottom surface of the caliber 1a is caused by rolling force, by forming a recess in the middle part of the roll main body 1 or in the 50 corresponding position of the roll shaft 2, and deflecting the roll by the vertical components of the surface pressure while rolling, thereby generating a compressive stress on the bottom surface of the caliber 1a. That is a bending stress is generated in the bottom section of the caliber 1a by rolling reaction, and this bending stress acts as a compressive stress on the bottom surface of the caliber 1a, and by this compressive stress, the tensile stress maximum value  $\sigma_{tmax}$  is reduced, hence preventing breakdown.

However, even by the method of forming a recess in the middle part of the roll main body 1 or in its corresponding position of the roll shaft 2, cracking and roll breakdown could not be sufficiently prevented owing to the following reasons.

FIG. 2 shows an example of roll peripheral direction distribution of vertical component (roll reaction) P of surface pressure applied to the caliber roll of a cold

Pilger rolling mill forming a caliber gradually decreasing in the radius in the peripheral direction, mean tensile stress  $\sigma_H$  of caliber bottom section and tensile stress  $\sigma_T$  of caliber bottom surface (corresponding to  $\sigma_{tmax}$  in FIG. 1) caused by it, in which the axis of abscissas denotes the position in the roll peripheral direction, and the axis of ordinates is the roll reaction and tensile stress. That is, according to this diagram, the roll reaction P reaches the maximum near section No. 0.3 in the roll peripheral position, the mean tensile stress  $\sigma_H$  reaches the maximum nearly at the maximum position of the roll reaction P, and the tensile stress  $\sigma_T$  of caliber bottom surface reaches the maximum nearly at section No. 0.55.

The reason of deviation of the maximum position of the tensile stress  $\sigma_T$  of caliber bottom surface in the rightward direction or in the caliber radius decreasing direction, with respect to the roll reaction maximum position, is as follows. The mean tensile stress  $\sigma_H$  increases as the roll reaction becomes larger, but even at the same roll reaction, as the caliber radius becomes smaller, the two, as shown in the diagram, the maximum position of the tensile stress  $\sigma_T$  of caliber bottom surface increases due to stress concentration, and by the effects of the tensile stress  $\sigma_T$  of caliber bottom surface is deviated to the smaller caliber radius side. Meanwhile, the multiple breakdown forming region of the caliber roll for rolling in the diagram coincides with the maximum position of the tensile stress  $\sigma_T$  of caliber bottom surface.

In the caliber roll for rolling showing such distribution, when the above recess forming technology is applied, the compressive stress generated on the roll caliber bottom surface depends on the roll reaction force itself and therefore the compressive force generated at the maximum position of the tensile stress of caliber bottom surface is smaller than the compressive stress generated at the maximum position of the roll reaction, and hence the effect by the compressive stress at the maximum position of the tensile stress of caliber bottom surface is small, thereby leading to roll breakage.

The material of the roll main body of the caliber roll for rolling is explained below.

Conventionally, the roll main body of caliber roll for rolling was generally made of SUJ5 steel specified as bearing steel in JIS, or high carbon low alloy tool steel such as 0.8% C-1.7% Cr-0.3% Mo-0.1% V steel (hereinafter the percentage expressing the content of components is wt. %). However, the high carbon low alloy steels are not sufficient in hardening, and large fluctuations of hardness due to uneven hardening and mass effect, and are likely to cause wear and cracking depending on application conditions. For hardening, therefore, instead of hardening the entire section of the roll, a technique called cored (surface) hardening for hardening only the surface layer by special heat treatment has been employed. In the roll fabricated by cored hardening, since the hardened portion is only the surface layer, the abrasion resistance is maintained only for a short term, and when the caliber surface layer is worn to a certain extent, the hardness of the caliber surface suddenly drops, thereby leading to collapse of the caliber shape.

Accordingly, as the material of the roll main body, the JIS SKD11 steel (high carbon high alloy tool steel) with excellent hardenability has come to be used. The roll made of this high carbon high alloy tool steel is excellent in hardenability and can be hardened entirely,

and special treatment such as cored hardening is not needed. However, the roll main body made of SKD11 steel is required to have a hardness of  $HRC$  60 or more (Rockwell C scale) from the viewpoint of prevention of caliber abrasion and surface spalling. To endow with such hardness, however, as clear from the tempering temperature curve in FIG. 3, for example, after hardening at  $1030^{\circ}C$ , tempering must be done at a low temperature of about  $200^{\circ}C$ . Accordingly, the subsequent heating temperature range is limited, and not only the temperature control is difficult at the time of shrinkage-fitting to the roll shaft, but also softening may be possibly caused by processing heat or abrasion heat in rolling. Furthermore, this SKD11 steel is not sufficient in toughness, and when applied in the roll main body, it is indicated that the caliber is likely to be broken from the bottom during rolling.

In this background it was once proposed to use a cold tool steel (C: 0.75 to 1.75%, Si: 3.0% or less, Mn: 0.1 to 2.0%, P: 0.020% or less, S: 0.003% or less, Cr: 5.0 to 11.0%, Mo: 1.3 to 5.0%, V: 0.1 to 5.0%, N: 0.020% or less, O: 0.0030% or less) with an attempt to enhance the toughness while maintaining the high hardness of the SKD11 steel, on the basis of the SKD11 steel, by decreasing the contents of P, S, and N, and increasing the content of Mo (Japanese Patent Application Laid-Open No. 64-11945). This steel (hereinafter called SKD11 modified steel) is superior to SKD11 steel in toughness, realizes the tempering effect by heating at  $450^{\circ}C$  or higher, and easy in temperature control in shrinkage-fitting, and free from risk of softening due to processing heat during use, but the following problems are known.

That is, the SKD11 modified steel (the cold tool steel disclosed in the Japanese Patent Application Laid-Open No. 64-11945). This steel (hereinafter called SKD11 by allowing to be used at high hardness by the portion of the superior toughness, and accordingly when applied in the roll main body of the caliber roll for rolling, the appropriate hardness is said to be  $HRC$  62 to 63. However, if a high impact load is applied as in the caliber roll for rolling, even by application of the SKD11 modified steel, it is difficult to prevent cracks from the caliber bottom, and this tendency is more obvious when used at such high hardness.

Besides, in this SKD11 modified steel, in order to maintain the material hardness of  $HRC$  62 or 63, the tempering temperature must be  $490^{\circ}$  to  $530^{\circ}C$ . in the case of  $1030^{\circ}C$ . hardening, but as clear from FIG. 3 this is the temperature range before and after the secondary hardening temperature, and even in this temperature range, if exceeding the secondary hardening temperature, the hardness drops suddenly, and such hardness cannot be maintained stably. Therefore, usually, the tempering temperature is below the secondary hardening temperature, and the tensile residual stress of the surface layer (generated as the surface shrinks at the time of cooling when hardening) and residual austenite (expanding by martensiting with the lapse of time) are not eliminated, thereby leaving the factors of cracks.

Thus, in the conventional caliber roll for rolling, the roll wear was excessive, and it was required to adjust the roll gap (adjust the outside diameter) frequently depending on the extent of roll wear, and to prepare the mandrels differing in size (adjust the product wall thickness), and short life of the roll and other problems were not sufficiently solved.

## SUMMARY OF THE INVENTION

The present inventors intensively researched, from such viewpoint, in order to present a caliber roll for rolling having a sufficiently satisfactory life (crack life, wear life), and realize tube making works without requiring frequent tasks for product size adjustment or preparation of mandrels in multiple sizes, and obtained the following findings.

That is, the SKD11 steel and SKD11 modified steel which are superior in hardening operation and abrasion resistance to other existing materials and are easy to obtain among cold tool steels are, when used as the material for the roll main body of the caliber roll for rolling, indeed likely to cause large cracks if prepared at high hardness according to the conventional tempering standard as mentioned above, and likely to cause wear, spalling and cracking if prepared at low hardness.

Nevertheless, such "large cracks" do not depend on

the hardness alone, but are also largely influenced by the material metal flow, residual stress and residual asutene. Therefore, by positively controlling the metal flow in the roll shaft central direction, and tempering after hardening in a temperature range above the secondary hardening temperature (see FIG. 3), effects of nonmetallic inclusions and giant carbides along the metal flows may be suppressed, and the residual stress is eliminated by high temperature tempering, and moreover as shown in FIG. 4 the residual austenite is lost, and the crack tendency is extremely lowered. In addition, when tempered at high temperature above the secondary hardening temperature, the hardness is reduced to  $HRC$  52 to 56, but the wear resistance is not practically so lowered as compared with that at  $HRC$  57 to 63 achieved in the treatment conforming to the conventional tempering standard.

Accordingly, selecting the SKD11 steel and SKD11 modified steel as the materials, by setting up positive measures for controlling the metal flow in the roll shaft central direction, and tempering at high temperature above the secondary hardening temperature after hardening to adjust the hardness in a range of  $HRC$  52 to 56, it is possible to realize a caliber roll for rolling possessing sufficient crack resistance and wear resistance, being free from adverse effects at the time of shrinkage-fitting to the roll shaft and risk of softening by processing heat and abrasion heat in rolling.

It is hence an object of the invention to present a caliber roll for rolling possessing excellent wear resistance and crack resistance and a manufacturing method of making its roll main body.

It is other object of the invention to present a caliber roll for rolling that is easy to handle and long in service life and a manufacturing method of making its roll main body.

It is another object of the invention to present a caliber roll for rolling at low cost and a manufacturing method of making its roll main body.

The caliber roll for rolling of the invention comprises a roll main body having a caliber on the outer circumference and possessing a shaft hole penetrating in the axial direction, and a roll shaft inserted in the shaft hole of the roll main body, in which the compressive stress in the widthwise direction of the roll main body is applied to the bottom of the caliber. When the compressive stress in the widthwise direction of the roll main body is applied thus to the bottom of the caliber of the roll main body, the maximum value of the tensile stress of the

caliber bottom surface which causes cracking or breakdown is lowered.

This compressive stress is applied by tapering either the internal circumference of the roll main body or the circumference of the roll shaft, and shrinkage-fitting or cold-fitting the roll main body and roll shaft. Alternatively the compressive stress is applied by pressing both end faces of the roll main body in the widthwise direction by means of a pressing jig fixed on the roll shaft.

A recess gap is disposed in either widthwise central internal circumference of the roll main body or its corresponding circumference of the roll shaft, or in both. By deflection of the roll by this recess gap, the compressive stress is generated in the bottom part of the caliber of the roll main body, and a greater compressive stress is applied to the bottom of the caliber of the roll main body.

The roll main body is made of an iron-based alloy including, by weight, C: 0.75 to 1.75%, Si: 3.0% or less, Mn: 2.0% or less, P: 0.030% or less, S: 0.030% or less, Cr: 5.0 to 13.00%, Mo: 0.80 to 5.0%, and V: 0.1 to 0.5%, and the entire hardness is adjusted to  $H_{RC}$  52 to 56, and it possesses a metal flow in the axial direction. The reasons for defining the chemical composition of the iron-based alloy as the material for the roll main body, the entire hardness of the roll main body, and the direction of metal flow as mentioned above are explained below.

The material steel used in the roll main body of the caliber roll for rolling is, for the sake of availability, desired to be in a composition range corresponding to the JIS SKD11 steel including C: 1.40 to 1.60%, Si: 0.40% or less, Mn: 0.60% or less, P: 0.030% or less, S: 0.030% or less, Cr: 11.00 to 13.00%, Mo: 0.80 to 1.20%, and V: 0.20 to 0.50%, and also allowable components such as Ni as required. Also from the viewpoint of maintaining the toughness, reducing P, S, O and N from the above composition, it is more preferable to define in the composition range of the SKD11 modified steel including C: 0.75 to 1.75%, Si: 3.0% or less, Mn: 0.1 to 2.0%, P: 0.020% or less, S: 0.003% or less, Cr: 5.0 to 11.0%, Mo: 1.3 to 5.0%, V: 0.1 to 0.5%, N: 0.020% or less and O: 0.0030% or less.

C, aside from heightening the hardness of martensite, acts to improve the wear resistance by forming a carbide together with Cr, Mo and V, but if its content is less than 0.75%, the desired effect by such action is not expected, or if contained more than 1.75%, the toughness is lowered, and hence the content of C is defined within 0.75 to 1.75%. Si is a useful component as a deoxidizer of steel, and at the same time it is effective for increasing the hardness of high temperature tempering. If contained excessively, however, the hot processability and toughness are lowered, and the upper limit of the Si content is defined at 3.0%. Mn is a useful component as a deoxidizing and desulfurizing agent of steel, and at the same time it is also effective for improvement of hardenability. If contained excessively, however, the processability is lowered, and hence the upper limit of the Mn content is defined at 2.0%. As the P content increases, the toughness of steel is lowered, and the upper limit of the P content is defined at 0.030%. If the S content is excessive, the impact value of the steel declines, and the upper limit of the S content is defined at 0.030%. Cr is dissolved in the matrix in hardening to enhance the hardenability, and also forms a Cr carbide to improve the wear resistance, but if the content is less than 5.0%, the desired effect by its action is not ob-

tained, or if contained more than 13.00%, the toughness deteriorates, and hence the Cr content is defined within 5.0 to 13.00%. Mo is dissolved in the matrix in hardening and forms a carbide to improve the wear resistance, and also acts to enhance the hardening and tempering resistance, but if the content is less than 0.80%, the desired effect by its action is not expected, or if contained more than 5.0%, further improvement of the effect is not expected, but also the hot processability is lowered, and hence the Mo content is defined within 0.80 to 5.0%. V acts to prevent increase of size of austenite particles and form fine carbides to improve the wear resistance and hardenability of the steel, but if its content is less than 0.1%, the desired effect by its action is not obtained, or if contained more than 0.5%, the processability is lowered, and hence the V content is defined within 0.1 to 0.5%. Meanwhile, the iron-based alloy to be used may also contain trace elements such as Ni as components aside from those defined above.

The entire hardness of the roll main body must be adjusted within  $H_{RC}$  52 to 56. This is because if the hardness of the entire roll section is less than  $H_{RC}$  52, a sufficient wear resistance is not maintained for a long term and the desired service life is not guaranteed, or if the roll main body hardness exceeds  $H_{RC}$  56, the toughness is insufficient, and large cracks leading to discarding of the roll are likely to occur.

Types of wear of the caliber roll for rolling include the following. First is the wear due to speed difference in rolling between the tube to be rolled and the caliber of the roll main body. It is advanced gradually in a relatively long time, but when the hardness is less than  $H_{RC}$  52, this wear is promoted in a short time, and the gloss of the caliber surface is lost. Typical wears leading to discarding of the roll are pitting wear and spalling shown in FIG. 5, and tube end mark shown in FIG. 6. What is particularly serious is pitting wear and spalling, which are caused in the caliber positions contacting with the portion corresponding to the major axis portion of the ellipse of the tube given rotating and feeding after rolled nearly in an elliptical form. More specifically, this area locally has a high surface pressure, and when the hardness of the caliber surface is low and strength is insufficient, pitting wear or peeling crack is induced. The tube end mark is an indentation of the roll surface due to contact with the tube end seam (corner of tube end) at the time of rolling, and in an extreme case the caliber surface is inducted irregularly in the circumferential direction, which adversely affects the surface properties and dimensional precision of the rolled tube.

On the other hand, the large crack, which leads to breakdown of the roll main body and is likely to occur when the roll main body hardness is set above  $H_{RC}$  56, causes shortness of the roll life. Generally, elevation of the roll hardness brings about a favorable effect for the wear resistance and fatigue strength improvement, but it induces cracks due to shortage of toughness, possibly leading to a shorter life in many cases. That is, the ordinary cold tube rolling (Pilger rolling) itself is an intermittent action, and excessive processing may occur due to abnormal feeding, or the mandrel may be broken and get into the rolling direction, and an impulsive overload due to such troubles are hard to avoid, and when the toughness is insufficient, a large crack is formed in such a case. Also, in order to raise the hardness of the roll main body to such a high value as mentioned above, the heat treatment (tempering) temperature must be low-

ered, which may lead to residual stress or residual austenite, resulting in a large crack.

Accordingly, by adjusting the hardness of the roll main body in a range of  $HRC$  52 to 56, the amount of abrasion becomes  $\frac{1}{2}$  or less of the conventional 0.8% C-1.7% Cr-0.3% Mo-0.1% V steel, and large cracks of the roll main body are almost completely eliminated. Still more, in this hardness region, tempering may be performed above the secondary hardening temperature, so that the problems of residual stress and residual austenite may be solved almost thoroughly.

Furthermore, in the roll main body, the direction of metal flow is also extremely important. That is, if there is no nonmetallic inclusion or giant carbide at all in the material for composing the roll main body, the direction of metal flow is not so important, but it is practically impossible that nonmetallic inclusions and giant carbides are completely absent. These nonmetallic inclusions and giant carbides are rolled in the direction (direction of metal flow) in which the material is rolled by rolling, forging and other processing. If the nonmetallic inclusion rolled in the direction of metal flow is present in a form of extended in the roll radial direction on the bottom surface of the caliber 1a of the roll main body 1 or immediately beneath it as shown in FIG. 7(a), a crack is initiated from it due to the tensile force (the tearing stress of the caliber bottom by the tube to be rolled) in the widthwise direction of the roll main body 1 when rolling. Therefore, if the inevitably existing nonmetallic inclusions and giant carbides are rolled, in order that the direction may be the widthwise direction (that is, the axial direction) of the roll main body 1 as shown in FIG. 7(b), the metal flow must be positively controlled in the axial direction.

The manufacturing method of according to roll main body of caliber roll for rolling of the invention comprises a step of fabricating a columnar material of specified outside diameter by screwing down a billet made of iron-based alloy with the above chemical composition from the radial direction, a step of spheroidizing the fabricated columnar material by holding at 830° to 880° C. for three hours or more, a step of cutting out a disc in a specified width from the spheroidized material, and cutting and forming a hole in the shaft axial direction of the disc and a caliber in the outer circumference, and a step of hardening at 1000° to 1050° C., and tempering by cooling in air while holding at 540° to 590° C. for an hour or more. The reasons for defining the conditions for the spheroidizing process, hardening process and tempering process are explained below.

The purpose of spheroidizing is to remove the processing strain, and if the heating temperature is held under 830° C. for less than three hours, the processing strain is not removed sufficiently, or heating in a temperature range exceeding 880° C. promotes production of giant carbides, which is not desired. If the hardening temperature is less than 1000° C., sufficient hardening effect is not obtained, or if the hardening temperature exceeds 1050° C., the texture becomes coarse, and the toughness is lowered. Tempering is the heat treatment for adjusting the hardness to  $HRC$  52 to 56, and if the tempering temperature is out of the range of 540° to 560° C., or if the tempering time is less than an hour, the desired hardness is not obtained.

The above and further objects and features of the invention will more fully be apparent from the following detailed description with accompanying drawings.

#### BRIEF DESCRIPTION OF THE DRAWINGS

FIG. 1 is an explanatory diagram showing the distribution of tensile stress  $\sigma_T$  acting on the caliber bottom surface of a caliber roll for rolling by surface pressure  $P$ .

FIG. 2 is a diagram showing an example of roll peripheral distribution of vertical components of surface pressure applied on a caliber roll for rolling and tensile stress of caliber caused by it.

FIG. 3 is a diagram showing a tempering temperature curve of high carbon high alloy tool steel.

FIG. 4 is a graph showing the relation of tempering temperature, number of times of tempering and residual austenite amount of high carbon high alloy tool steel.

FIG. 5 is a conceptual diagram explaining the situation of pitting wear and spalling of a caliber roll for rolling.

FIG. 6 is a conceptual diagram explaining the situation of tube end mark occurrence of a caliber roll for rolling.

FIG. 7 is a conceptual diagram explaining the situation of metal flow direction and nonmetallic inclusion of a caliber roll for rolling.

FIG. 8 is a conceptual diagram explaining a processing method of a billet relating to the invention.

FIG. 9 is a schematic diagram showing the entire shape of a roll main body of a caliber roll for rolling.

FIG. 10 is a schematic diagram showing an example of a shape of the roll main body of a caliber roll for rolling.

FIG. 11 is a schematic diagram showing an example of another shape of the roll main body of a caliber roll for rolling.

FIG. 12 is a schematic diagram showing an embodiment of a caliber roll for rolling of the invention.

FIG. 13 is a schematic diagram showing another embodiment of a caliber roll for rolling of the invention.

FIG. 14 is a schematic diagram showing a further embodiment of a caliber roll for rolling of the invention.

FIG. 15 is a schematic diagram showing a further different embodiment of a caliber roll for rolling of the invention.

FIG. 16 is an explanatory diagram showing a generation mechanism of compressive stress at the time of shrinkage-fitting (or cold-fitting) of roll main body and roll shaft.

FIG. 17 is an explanatory diagram showing another generation mechanism of compressive stress at the time of shrinkage-fitting (or cold-fitting) of roll main body and roll shaft.

FIG. 18 is a schematic diagram showing an embodiment of generating compressive stress by a pressure ring.

FIG. 19 is a schematic diagram showing another embodiment of generating compressive stress by a pressure ring.

FIG. 20 is a schematic diagram showing a reference example to a caliber roll for rolling of the invention.

FIG. 21 is a schematic diagram showing another reference example to a caliber roll for rolling of the invention.

#### DESCRIPTION OF THE PREFERRED EMBODIMENTS

Some of the embodiments of the invention are described in detail below.

First the manufacturing method of the roll main body of a caliber roll for rolling is explained.

In manufacturing the roll main body of a caliber roll for rolling relating to the invention, first is prepared a billet (ingot) of an iron-based alloy steel including, by weight, C: 0.75 to 1.75%, Si: 3.0% or less, Mn: 2.0% or less, P: 0.030% or less, S: 0.030% or less, Cr: 5.0 to 13.00%, Mo: 0.80 to 5.0%, and V: 0.1 to 0.5%. This billet may be obtained by melting the steel having the above chemical composition in, for example, an electric furnace, but, if possible, it is preferable to use a columnar ingot by melting in an electric furnace to obtain a columnar piece as an electrode, and further processing by electroslag remelting (ESR). That is, by ESR process, segregation is eliminated as far as possible, and the size of giant carbide is reduced, and the number thereof is also decreased, and moreover nonmetallic inclusions decrease and the fatigue strength is raised, so that the crack resistance is further enhanced.

In succession, this billet is rolled in the axial direction by applying pressure from the radial direction (the direction of arrow A in FIG. 8) by rolling or forging, thereby obtaining a columnar material. As a result, the direction of metal flow is the axial direction as indicated by arrow B in FIG. 8. Thus, the metal flow in the axial direction is realized by screwing down the casting material from the radial direction by rolling or forging with a sufficient reduction into a columnar shape, when obtaining a columnar material for fabricating the roll main body. At this time, the elongation ratio (the sectional area before processing/sectional area after processing) should be preferably four times or more in order to produce a sufficient metal flow.

Sequentially, such columnar material is cut in slices, and a disc-shaped roll material is obtained, but prior to this the columnar material is spheroidized by holding at 830° to 880° C. for three hours or more and cooling a 35 furnace. The purpose of this spheroidizing is to remove processing strains, and if the holding time of the heating temperature of below 830° C. is less than three hours, the processing strains are not removed sufficiently, or heating in a temperature range exceeding 880° C. promotes formation of giant carbides, which is not preferable. In thus prepared material, the direction of the metal flow is the widthwise direction (the axial direction), thereby obtaining, needless to say, the anisotropy resistant to cracks.

Meanwhile, as the technique for preparing a disc material for manufacturing one roll main body, for example, the columnar ingot is directly cut in slices, and obtained short columnar ingots are forged and screwed down in the direction to widen the diameter. In this case, however, the metal flow direction is the radial direction of the disc material, and therefore the nonmetallic inclusions and giant carbides are rolled in the radial direction, and the roll main body manufactured therefrom is likely to be cracked by the tensile force applied to the caliber bottom at the time of rolling, which is not preferable.

Next, in the disc material, as shown in FIG. 9, a tapered caliber 1a is cut and formed, and the lateral face and circumferential face are aligned by cutting. Furthermore, a shaft hole 1b for shrinkage-fitting (or cold-fitting) to the roll shaft is pierced in the axial direction, thereby completing the roll main body 1.

Thus prepared roll main body 1 is then treated by hardening and tempering.

The hardening process is executed in order to transform the material texture into martensite texture to obtain high hardness, and after heating to 1000° to 1050°

C., the material is cooled in air or cooled in oil. As a result, the hardness of about H<sub>RC</sub> 63 is obtained. At this step, if the hardening temperature is less than 1000° C., a sufficient hardening effect is not achieved, or if the hardening temperature exceeds 1050° C., the texture is made coarse, and the toughness is lowered.

Tempering is a heat treatment for adjusting the hardness to H<sub>RC</sub> 52 to 56, and it is executed in the condition of holding at 540° to 590° C. for an hour or more and cooling in air. If the tempering temperature is out of the above range, or the tempering time is less than an hour, adjustment to the desired hardness is unstable. Here, the tempering temperature is to select a proper temperature in this temperature range depending on the steel grade and hardening condition to adjust the hardness to H<sub>RC</sub> 52 to 56, and when the SKD11 steel is hardened at 1030° C. and cooled in air, it is desired to temper at 540° to 560° C., or when the SKD11 modified steel is hardened at 1030° C. and cooled in air, at 560° to 580° C., or when hardened at 1030° C. and cooled in oil, at 570° to 590° C.

As known, meanwhile, from the tempering temperature curve in FIG. 3, once the hardness is determined, the tempering temperature is decided accordingly, and in the tempering of the invention, this temperature is above the secondary hardening temperature. Besides, since the tempering temperature is set at a high temperature above the secondary hardening temperature, the residual austenite is decomposed and is almost completely lost, and the tensile residual stress is easily released. Incidentally, it is desired to temper plural times. That is, as is clear from FIG. 4 showing the relation of the tempering temperature, number of times of tempering and residual austenite, it is intended to decrease the residual austenite furthermore.

The roll main body 1 after hardening and tempering is entirely ground and finished to correct the shape strain by hardening and tempering, adjust the roughness of caliber, and achieve the dimensional precision, and a product is obtained.

Explained below is the shape of the roll main body of a caliber roll for rolling of the invention and the roll shaft to be inserted therein, for producing a compressive stress in the bottom of the caliber of the roll main body, in detail.

FIGS. 10 and 11 are schematic diagrams showing the types of roll main body 1. The example shown in FIG. 10 is the roll main body 1 of the type having a specified caliber 1a formed on the outer circumference and a shaft hole 1b pierced in its axial direction. The example shown in FIG. 11 is the roll main body 1 of the type having a specified caliber 1a formed on the outer circumference and a shaft hole 1b pierced in its axial direction, and further having a recess gap 1c in the middle of the shaft hole 1b being contiguous thereto. In FIGS. 10 and 11, W, D, d respectively denote the width of the roll main body 1, the outside diameter of the roll main body 1, and the inside diameter of the roll main body 1 (the diameter of shaft hole 1b), and L in FIG. 11 represents the length of the recess gap 1c in the widthwise direction.

FIGS. 12 to 15 are schematic diagrams showing examples of roll main body 1 and roll shaft 2 of the caliber roll for rolling of the invention, and a part of the roll main body 1 is omitted. In each example, a shrinkage-fitting allowance (or cold-fitting allowance) 1d is disposed at the inner circumferential side of the roll main body 1, and this shrinkage-fitting allowance (or cold-fitting allowance) 1d is large at both sides of the roll main body

1 in the width direction, and gradually decreases toward the central part. The shrinkage fitting allowance can be provided by forming first and second tapered sections on either the roll main body 1 or on the roll shaft 2, the first and second tapered sections converging towards a central part of the roll main body (i.e., the first and second tapered sections have diameters which either increase or decrease as the tapered sections become closer together in the axial direction), as shown in FIGS. 12-17. Each embodiment is individually described below.

FIG. 12 relates to a caliber roll for rolling including a roll main body 1 having a caliber 1a and a shaft hole 1b of uniform diameter and provided with a shrinkage-fitting allowance (or cold-fitting allowance) 1d, and a roll shaft 2 of which diameter gradually decreases in a taper from both ends toward the central part. In the case of this caliber roll for rolling, when the roll main body 1 and roll shaft 2 are shrinkage-fitted (or cold-fitted), a compressive stress is built up in the bottom of the caliber 1a of the roll main body 1 due to the taper action of the roll shaft 2.

FIG. 13 shows a caliber roll for rolling including a roll main body 1 having a caliber 1a and a shaft hole 1b of which diameter increases in a taper toward the central part and provided with a shrinkage-fitting allowance (or cold-fitting allowance) 1d, and a roll shaft 2 of uniform diameter. In the case of this caliber roll for rolling, too, by shrinkage-fitting (or cold-fitting) of the two, a compressive stress is generated in the bottom of the caliber 1a same as in the embodiment shown in FIG. 12.

FIG. 14 shows a caliber roll for rolling including a roll main body 1 having a caliber 1a and a shaft hole 1b of uniform diameter, and provided with a recess gap 1c in the middle part of the shaft hole 1b and a shrinkage-fitting allowance (or cold-fitting allowance) 1d, and a roll shaft 2 of which diameter decreases gradually in a taper from both ends toward the central part. In this case, a compressive stress due to shrinkage-fitting allowance (or cold-fitting allowance) 1d, and a compressive stress generated due to deflection of the roll by recess gap 1c are produced in the bottom of the caliber 1a.

FIG. 15 shows a caliber roll for rolling including a roll main body 1 having a caliber 1a and a shaft hole 1b of which diameter increases in a taper toward the central part, and provided with a recess gap 1c in the middle part of the shaft hole 1b and a shrinkage-fitting allowance (or cold-fitting allowance) 1d, and a roll shaft 2 of uniform diameter. In this case, too, just as in the embodiment shown in FIG. 14, both compressive force due to shrinkage-fitting allowance (or cold-fitting allowance) 1d and compressive stress due to deflection of roll by recess gap 1c are generated in the bottom of the caliber 1a.

Here is explained the mechanism of generation of compressive stress due to shrinkage-fitting (or cold-fitting) in the case of taper processing of the internal circumference of the roll main body 1. As shown in FIGS. 16 and 17, the shrinkage-fitting allowance (or cold-fitting allowance) has the minimum value  $\delta_{min}$  in the center of the roll main body 1 in the widthwise direction, and the maximum value  $\delta_{max}$  at both ends, and when shrinkage-fitting (cold-fitting) is executed, the roll main body 1 is deformed as indicated by broken line, and a compressive stress is applied to the bottom of the caliber 1a.

The method of determining the shrinkage-fitting allowance (or cold-fitting allowance) is described below.

1. Mean shrinkage-fitting allowance (or cold-fitting allowance)  $\delta_{mean}$

5 In the case of a conventional caliber roll for Pilger rolling (without taper processing and recess gap in the roll main body), in order to prevent slipping of the roll main body and roll shaft, the shrinkage-fitting force (or cold-fitting force) is set as design specification, and the shrinkage-fitting allowance (or cold-fitting allowance) is predetermined to maintain this shrinkage-fitting force (or cold-fitting force). Therefore, if the shrinkage-fitting allowance (or cold-fitting allowance) is, for example as shown in FIG. 16,  $\delta_{max}$  at both sides of the roll main body 1, and  $\delta_{min}$  in the central part, the mean shrinkage-fitting allowance (or cold-fitting allowance)  $\delta_{mean} = (\delta_{max} + \delta_{min})/2$  is so set as to be greater than the predetermined shrinkage-fitting allowance (or cold-fitting allowance).

10 2. Maximum shrinkage-fitting allowance (or cold-fitting allowance)  $\delta_{max}$

The roll main body and roll shaft are made of, for example, JIS-SKD11 steel, and the strength is adjusted by final hardening and tempering, and the tempering temperature is about 250°C. at the lowest although variable with the grade of steel. At the time of shrinkage-fitting, meanwhile, the roll main body heating temperature must not be above the tempering temperature, and to prevent softening of the surface of the roll main body, it is desired to set at a temperature of 200°C. or less. Therefore, the maximum shrinkage-fitting allowance (or cold-fitting allowance)  $\delta_{max}$  is based on the thermal expansion allowance by heating of the roll main body (or shrinkage allowance by cooling of the roll shaft), and is determined in consideration of the working efficiency and other conditions.

15 3. Minimum shrinkage-fitting allowance (or cold-fitting allowance)  $\delta_{min}$

Once the mean shrinkage-fitting allowance (or cold-fitting allowance)  $\delta_{mean}$  and maximum shrinkage-fitting allowance (or cold-fitting allowance)  $\delta_{max}$  are determined,  $\delta_{min}$  is calculated in the following formula.

$$\delta_{min} = 2 \delta_{mean} - \delta_{max}$$

20 By thus determining  $\delta_{max}$ ,  $\delta_{min}$ , in order to achieve  $\delta_{max}$  at both ends of the roll main body and  $\delta_{min}$  in the central part, the inner circumference of the roll main body 1 or the circumference of the roll shaft 2 is tapered. Alternatively, as shown in FIG. 17, in the case of a caliber roll for rolling having a recess gap 1c in the middle of the roll main body 1, since the recess gap 1c is not responsible for maintaining the shrinkage-fitting force (or cold-fitting force) at the time of shrinkage-fitting (or cold-fitting), the mean shrinkage-fitting allowance (or cold-fitting allowance)  $\delta_{mean}$  at both sides is taken sufficiently depending on the width of the recess gap 1c, and the maximum shrinkage-fitting allowance (or cold-fitting allowance)  $\delta_{max}$  and minimum shrinkage-fitting allowance (or cold-fitting allowance)  $\delta_{min}$  are determined.

25 60 65 When the shrinkage-fitting allowance (or cold-fitting allowance) is determined in this way, the flange part of the roll main body 1 is tilted in the direction of the caliber 1a depending on the taper angle ( $\alpha$  in FIG. 16,  $\beta$  in FIG. 17) of the shrinkage-fitting allowance (or cold-fitting allowance), and a compressive stress  $\sigma_A$  corre-

sponding to the taper angle  $\alpha$ ,  $\beta$  acts on the bottom of the caliber 1a. Incidentally, as a result of thus determining the taper angle of the shrinkage-fitting allowance (or cold-fitting allowance), the compressive stress  $\sigma_A$  acting on the bottom of the caliber 1a becomes large, and accordingly the tensile stress  $\sigma_B$  acting on the middle of the inner circumference of the roll main body 1 also becomes large. Consequently, the value of subtracting the preliminarily applied compressive stress  $\sigma_A$  from the maximum tensile stress  $\sigma_{Tmax}$  acting on the bottom surface of the caliber 1a during rolling may be sometimes smaller than the tensile stress  $\sigma_B$  acting on the middle of the inner circumference of the roll main body 1. In such state, although roll cracking from the bottom of the caliber 1a may be prevented, since the tensile stress  $\sigma_B$  is great, roll cracking may be initiated from the middle of the inner side of the roll main body 1. At this time, the taper angle of the shrinkage-fitting allowance (or cold-fitting allowance) is reduced so that the value of subtracting  $\sigma_A$  from  $\sigma_{Tmax}$  may be about  $\sigma_B$ . In the case of a caliber roll for rolling having a recess gap 1c contiguous to the shaft hole 1b, as mentioned above, a compressive stress acts on the bottom of the caliber 1a by deflection of the roll main body 1 due to the recess gap 1c. If the result of subtracting the sum of this compressive stress and the compressive stress caused by the taper angle of the shrinkage-fitting allowance (or cold-fitting allowance) from  $\sigma_{Tmax}$  is smaller than  $\sigma_B$ , the taper angle should be reduced.

In other embodiments explained below, it is intended to apply a compressive stress to the bottom of the caliber 1a of the roll main body 1 by a pressing jig. FIGS. 18 and 19 are schematic diagrams of such embodiments of a caliber roll for rolling. FIG. 18 relates to an exam-

5 threads 2a of the roll shaft 2, so that a compressive force is applied to the bottom of the caliber 1a.

In the embodiments shown in FIGS. 18 and 19, the recess gap 1c is provided, but it is not always necessary.

Actual manufactured examples of the caliber roll for rolling of the invention and their performances are described specifically below.

First, in an electric furnace, steels of various chemical compositions are melted, and columnar ingots of 800 mm $\phi$  in outside diameter are obtained. Some of the samples are prepared in columnar ingots in the same size by further electroslag remelting. The columnar ingots are forged by screwing down only in the radial direction, and columnar materials of 310 mm $\phi$  in outside diameter are obtained, and the obtained columnar materials are spheroidized in various conditions, and cut in slices, and disc materials of 140mm in width are obtained. In succession, a taper caliber is formed in the disk material by cutting and processing, and the lateral surface and circumferential surface are properly treated, and a shaft hole is pierced in the axial direction in order to shrinkage-fit the roll shaft. After hardening and tempering in various conditions, the whole surface is ground, and a roll main body with the outside diameter of 300 mm $\phi$  and width of 130 mm is obtained. Needless to say, the metal flow of the roll main body manufactured is in the axial direction.

In this manufacturing process, three iron-based alloy steels having the chemical compositions as shown in Table 1 are used as the material steels. Steel grades A and B in Table 1 are the desired steels of the invention, and in particular steel grade B is the SKD11 modified steel, while steel grade C in Table 1 is a reference steel.

TABLE 1

| Steel grade            | Chemical composition |      |      |      |       |      |     |      |      |       |         | Fe and impurities |
|------------------------|----------------------|------|------|------|-------|------|-----|------|------|-------|---------|-------------------|
|                        | C                    | Si   | Mn   | P    | S     | Cr   | Mo  | V    | N    | O     |         |                   |
| <u>Invention steel</u> |                      |      |      |      |       |      |     |      |      |       |         |                   |
| A                      | 1.60                 | 0.31 | 0.40 | 0.02 | 0.01  | 12.0 | 0.9 | 0.26 | 0.02 | 0.004 | Balance |                   |
| B                      | 0.95                 | 1.04 | 0.41 | 0.01 | 0.001 | 8.4  | 2.0 | 0.24 | 0.01 | 0.002 | Balance |                   |
| <u>Reference steel</u> |                      |      |      |      |       |      |     |      |      |       |         |                   |
| C                      | 0.80                 | 0.28 | 0.37 | 0.02 | 0.01  | 1.7  | 0.3 | 0.11 | 0.02 | 0.004 | Balance |                   |

ple of using a roll main body 1 having a caliber 1a with the same shape in the peripheral direction, and FIG. 19 shows an embodiment of using a roll main body 1 having a caliber 1a with a taper in the peripheral direction.

FIG. 18 shows a caliber roll for rolling including a roll main body 1 having a caliber 1a with the same shape in the peripheral direction, and provided with a recess gap 1c, and a roll shaft 2 having male threads 2a formed at both ends. A round pressure ring 3 having a pressure head 3a corresponding to the bottom of the caliber 1a in the peripheral direction is screwed onto the male threads 2a of the roll shaft 2 together with a locknut 4, and a compressive force is applied to the bottom of the caliber 1a.

FIG. 19 shows a caliber roll for rolling including a roll main body 1 having a caliber 1a with a taper in the peripheral direction, and provided with a recess gap 1c, and a roll shaft 2 having male threads 2a formed at both ends. A non-round pressure ring 3 having a pressure head 3a corresponding to the bottom of the caliber 1a in the peripheral direction is externally fitted to the roll shaft 2, and is locked with a sink key 5 for correspondence of the pressure head 3a and the bottom of the caliber 1a, and a locknut 4 is screwed onto the male

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785

TABLE 3(a)

| Test No.    | Roll main body type | Caliber roll type | Shrinkage-fitting allowance (mm) |                 | Max. tensile stress caused during rolling (kgf/mm <sup>2</sup> ) |
|-------------|---------------------|-------------------|----------------------------------|-----------------|------------------------------------------------------------------|
|             |                     |                   | $\delta_{\max}$                  | $\delta_{\min}$ |                                                                  |
| 1 Reference | FIG. 10             | FIG. 20           | 0.110                            | 0.110           | 81                                                               |
| 2 Invention | FIG. 10             | FIG. 12           | 0.160                            | 0.060           | 81                                                               |
| 3 Reference | FIG. 11             | FIG. 21           | 0.120                            | 0.120           | 81                                                               |
| 4 Invention | FIG. 11             | FIG. 14           | 0.160                            | 0.080           | 81                                                               |
| 5 Invention | FIG. 10             | FIG. 19           | 0.110                            | 0.110           | 81                                                               |

TABLE 3(b)

| Test No.    | Compressive stress caused by recess deflection (kgf/mm <sup>2</sup> ) |                 | Compressive stress caused by taper shrinkage-fitting or pressing jig (kgf/mm <sup>2</sup> ) | Rolling length until discarding ( $\times 10^3$ m)                | Cause of discarding |
|-------------|-----------------------------------------------------------------------|-----------------|---------------------------------------------------------------------------------------------|-------------------------------------------------------------------|---------------------|
|             | $\delta_{\max}$                                                       | $\delta_{\min}$ |                                                                                             |                                                                   |                     |
| 1 Reference | 0                                                                     |                 | 0                                                                                           | 30-40                                                             | Crack               |
| 2 Invention | 0                                                                     |                 | 12                                                                                          | 100-120                                                           | Crack               |
| 3 Reference | 8                                                                     |                 | 0                                                                                           | 60-75                                                             | Crack               |
| 4 Invention | 8                                                                     |                 | 16                                                                                          | Even at 200 or higher, no crack is formed, being in normal state. |                     |
| 5 Invention | 0                                                                     |                 | 12                                                                                          | 100-120                                                           | Crack               |

TABLE 4(a)

| Test No.    | Roll main body type | Caliber roll type | Shrinkage-fitting allowance (mm) |                 | Max. tensile stress caused during rolling (kgf/mm <sup>2</sup> ) |
|-------------|---------------------|-------------------|----------------------------------|-----------------|------------------------------------------------------------------|
|             |                     |                   | $\delta_{\max}$                  | $\delta_{\min}$ |                                                                  |
| 1 Reference | FIG. 10             | FIG. 20           | 0.110                            | 0.110           | 81                                                               |
| 2 Invention | FIG. 10             | FIG. 12           | 0.160                            | 0.060           | 81                                                               |
| 3 Reference | FIG. 11             | FIG. 21           | 0.120                            | 0.120           | 81                                                               |
| 4 Invention | FIG. 11             | FIG. 14           | 0.160                            | 0.080           | 81                                                               |
| 5 Invention | FIG. 11             | FIG. 19           | 0.110                            | 0.110           | 81                                                               |

TABLE 4(b)

| Test No.    | Compressive stress caused by recess deflection (kgf/mm <sup>2</sup> ) |                 | Compressive stress caused by taper shrinkage-fitting or pressing jig (kgf/mm <sup>2</sup> ) | Rolling length until discarding ( $\times 10^3$ m)                | Cause of discarding |
|-------------|-----------------------------------------------------------------------|-----------------|---------------------------------------------------------------------------------------------|-------------------------------------------------------------------|---------------------|
|             | $\delta_{\max}$                                                       | $\delta_{\min}$ |                                                                                             |                                                                   |                     |
| 1 Reference | 0                                                                     |                 | 0                                                                                           | 100-120                                                           | Crack               |
| 2 Invention | 0                                                                     |                 | 12                                                                                          | 200-300                                                           | Crack               |
| 3 Reference | 8                                                                     |                 | 0                                                                                           | 150-250                                                           | Crack               |
| 4 Invention | 8                                                                     |                 | 16                                                                                          | Even at 500 or higher, no crack is formed, being in normal state. |                     |
| 5 Invention | 0                                                                     |                 | 12                                                                                          | 200-300                                                           | Crack               |

In Tables 3, 4, the caliber roll for rolling of same test number differs only in the hardness of its roll main body. In all caliber rolls for rolling in Table 3, the hardness of the roll main body is H<sub>RC</sub> 58, and in all caliber rolls for rolling in Table 4, the hardness of the roll main body is H<sub>RC</sub> 54. In all caliber rolls for rolling in Tables 3 and 4, the metal flow direction is the axial direction. The constructions of reference cases of test numbers 1, 3 in Tables 3, 4 are shown in FIGS. 20, 21, respectively. In both cases, the thickness of the shrinkage-fitting allowance 1d is uniform. In the example shown in FIG. 20, the roll shaft 2 of uniform diameter is inserted into the roll main body 1 having the caliber 1a and shaft hole 1b of uniform diameter, and in the example in FIG. 21, the roll shaft 2 of uniform diameter is inserted into the roll main body 1 having the caliber 1a and shaft hole 1b of uniform diameter and provided with the recess gap 1c contiguous to the shaft hole 1b.

As is clear from the results in Tables 3 and 4, in the case of the present invention embodiments (test numbers 2, 4) of applying compressive stress to the bottom of the caliber 1a of the roll main body 1 by combining

the tapered roll shaft 2 with the roll main body 1 having the shaft hole 1b of uniform diameter, or in the case of the present invention embodiment (test number 5) of applying compressive stress to the bottom of the caliber 1a of the roll main body 1 by means of a pressing jig (pressure ring 3), the roll life is about three or four times longer than that of the reference examples (test numbers 1, 3) without such compressive stress.

Besides, in each table, in the example (test number 4) of using the roll main body 1 having the recess gap 1c contiguous to the shaft hole 1b, the compressive stress caused by the action of the tapered roll shaft 2 is com-

bined with the compressive stress caused by deflection of the roll by this recess gap 1c, and therefore the roll life is extended as compared with the example (test number 2) using the roll main body 1 without recess gap 1c.

Furthermore, as understood from the comparison between Table 3 and Table 4, the roll life is longer when the entire hardness of the roll main body 1 is H<sub>RC</sub> 54 (Table 3), as compared with H<sub>RC</sub> 58 (Table 4).

Using steel grades A, B, C in Table 1 differing in chemical composition as the materials, caliber rolls for rolling are manufactured by further varying the tempering conditions, and the rolling is tested by using them in a rolling process, of which results are shown in Table 5.

In all caliber rolls for rolling in Table 5, the rolling conditions are the same as in Table 2, and the type of the roll main body 1 is the type of FIG. 10 free from compressive stress due to deflection of the roll without recess gap 1c, and the entire construction is the type of FIG. 20 free from compressive stress due to shrinkage-

fitting. The reference examples of test numbers 14, 15 are not forged, and the metal flow is not in the axial direction, while the metal flow is in the axial direction in all other examples.

Comparing the invention and reference examples in Table 5, it is easily seen that the caliber roll for rolling of the invention possesses an excellent life.

Furthermore, using the iron-based alloy having the chemical composition relating to the invention (specifi-

cally steel grade A or B in Table 1), and in the tempering conditions in the range of the invention, the caliber rolls for rolling of the type of causing compressive stress in the caliber are manufactured (specifically, the roll main body 1 is the type of FIG. 11, and the entire construction is the type of FIG. 14), and by these caliber rolls for rolling, the rolling process is conducted (the rolling conditions are the same as in Table 2). The rolling results are shown in Table 6.

TABLE 5(a)

| Test No.         | Roll material | OD of ingot (mm) | OD after forging (mm) | Spheroidizing condition              | Hardening condition                            | Tempering condition        |                |         |
|------------------|---------------|------------------|-----------------------|--------------------------------------|------------------------------------------------|----------------------------|----------------|---------|
| <u>Reference</u> |               |                  |                       |                                      |                                                |                            |                |         |
| 1                | A             |                  |                       |                                      | 520° C. × 6 hr                                 | 2 times                    |                |         |
| <u>Invention</u> |               |                  |                       |                                      |                                                |                            |                |         |
| 2                |               | No               |                       |                                      | 540° C. × 6 hr                                 | 2 times                    |                |         |
| 3                |               |                  |                       |                                      | 550° C. × 6 hr                                 | 2 times                    |                |         |
| 4                |               |                  |                       |                                      | 560° C. × 6 hr                                 | 2 times                    |                |         |
| <u>Reference</u> |               |                  |                       |                                      |                                                |                            |                |         |
| 5                |               |                  |                       |                                      | 570° C. × 6 hr                                 | 2 times                    |                |         |
| <u>Invention</u> |               |                  |                       |                                      |                                                |                            |                |         |
| 6                |               | Yes              |                       |                                      | 550° C. × 6 hr                                 | 2 times                    |                |         |
| <u>Reference</u> |               |                  |                       |                                      |                                                |                            |                |         |
| 7                | B             | 800              | 310                   | 850° C. × 5 hr<br>cooling in furnace | 1030° C.<br>cooling in air                     | 550° C. × 6 hr             | 2 times        |         |
| <u>Invention</u> |               |                  |                       |                                      |                                                |                            |                |         |
| 8                |               |                  |                       |                                      | 560° C. × 6 hr                                 | 2 times                    |                |         |
| 9                |               |                  |                       |                                      | 570° C. × 6 hr                                 | 2 times                    |                |         |
| 10               |               |                  |                       |                                      | 580° C. × 6 hr                                 | 2 times                    |                |         |
| <u>Reference</u> |               |                  |                       |                                      |                                                |                            |                |         |
| 11               |               |                  |                       |                                      | 590° C. × 7 hr                                 | 2 times                    |                |         |
| <u>Invention</u> |               |                  |                       |                                      |                                                |                            |                |         |
| 12               |               | Yes              |                       |                                      | 570° C. × 6 hr                                 | 2 times                    |                |         |
| <u>Reference</u> |               |                  |                       |                                      |                                                |                            |                |         |
| 13               | C             | No               |                       | 810° C. × 5 hr<br>cooling in furnace | 850° C.<br>cooling in oil<br>(cored hardening) | 250° C. × 3 hr             | 2 times        |         |
| 14               | A             | Yes              | 320                   | Not forged                           | 850° C. × 5 hr<br>cooling in furnace           | 1030° C.<br>cooling in air | 550° C. × 6 hr | 2 times |
| 15               | B             |                  |                       |                                      |                                                | 570° C. × 6 hr             | 2 times        |         |

TABLE 5(b)

| Test No.         | Product hardness (HRC) | Rolling length until discarding ( $\times 10^3$ m) | Cause of discarding | Remarks                                                     |
|------------------|------------------------|----------------------------------------------------|---------------------|-------------------------------------------------------------|
| <u>Reference</u> |                        |                                                    |                     |                                                             |
| 1                | 58                     | 20-60                                              | Crack               | Large crack (roll cutoff), short life, unstable             |
| <u>Invention</u> |                        |                                                    |                     |                                                             |
| 2                | 56                     | 70-120                                             | Crack               | Large crack decreases                                       |
| 3                | 54                     | 100-120                                            | Crack               | Favorable working efficiency                                |
| 4                | 52                     | 100-120                                            | Crack               | Favorable working efficiency                                |
| <u>Reference</u> |                        |                                                    |                     |                                                             |
| 5                | 51                     | 30-60                                              | Pitting wear        | Large wear, surface conditioning needed after about 20000 m |
| <u>Invention</u> |                        |                                                    |                     |                                                             |
| 6                | 54                     | 300 or more                                        | —                   | Favorable working efficiency                                |
| <u>Reference</u> |                        |                                                    |                     |                                                             |
| 7                | 58                     | 20-60                                              | Crack               | Large crack (roll cutoff), short life, unstable             |
| <u>Invention</u> |                        |                                                    |                     |                                                             |
| 8                | 56                     | 70-130                                             | Crack               | Large crack decreases                                       |
| 9                | 54                     | 100-120                                            | Crack               | Favorable working efficiency                                |
| 10               | 52                     | 100-120                                            | Crack               | Favorable working                                           |

TABLE 5(b)-continued

| Test No.         | Product hardness (HRC)    | Rolling length until discarding ( $\times 10^3$ m) | Cause of discarding | Remarks                                                                                                                   |
|------------------|---------------------------|----------------------------------------------------|---------------------|---------------------------------------------------------------------------------------------------------------------------|
| efficiency       |                           |                                                    |                     |                                                                                                                           |
| <u>Reference</u> |                           |                                                    |                     |                                                                                                                           |
| 11               | 51                        | 30-70                                              | Fitting wear        | Large wear, surface conditioning needed after about 20000 m                                                               |
| <u>Invention</u> |                           |                                                    |                     |                                                                                                                           |
| 12               | 54                        | 200 or more                                        | —                   | Favorable working efficiency                                                                                              |
| 13               | Surface: 58<br>Inside: 35 | 25-45                                              | Crack               | Crack, large crack occur in short time, wear is excessive, and sufficient surface conditioning needed after about 20000 m |
| <u>Reference</u> |                           |                                                    |                     |                                                                                                                           |
| 14               | 54                        | 10-40                                              | Crack               | Large crack (roll cutoff), short life, unstable                                                                           |
| 15               | 54                        | 10-40                                              | Crack               | Large crack (roll cutoff), short life, unstable                                                                           |

TABLE 6(a)

| Test No.         | Roll material | ESR | OD of ingot (mm) | OD after forging (mm) | Spheroidizing condition                  | Hardening condition     | Tempering condition   | Product hardness (HRC) |
|------------------|---------------|-----|------------------|-----------------------|------------------------------------------|-------------------------|-----------------------|------------------------|
| <u>Invention</u> |               |     |                  |                       |                                          |                         |                       |                        |
| 1                | A             |     |                  |                       |                                          |                         | 540° C. $\times$ 6 hr | 2 times                |
| 2                |               | No  | 800              | 310                   | 850° C. $\times$ 5 hr cooling in furnace | 1030° C. cooling in air | 550° C. $\times$ 6 hr | 2 times                |
| 3                |               |     |                  |                       |                                          |                         | 560° C. $\times$ 6 hr | 2 times                |
| 4                |               | Yes |                  |                       |                                          |                         | 550° C. $\times$ 6 hr | 2 times                |
| 5                | B             |     |                  |                       |                                          |                         | 560° C. $\times$ 6 hr | 2 times                |
| 6                |               | No  |                  |                       |                                          |                         | 570° C. $\times$ 6 hr | 2 times                |
| 7                |               |     | 800              | 310                   | 850° C. $\times$ 5 hr cooling in furnace | 1030° C. cooling in air | 580° C. $\times$ 6 hr | 2 times                |
| 8                |               | Yes |                  |                       |                                          |                         | 570° C. $\times$ 6 hr | 2 times                |

TABLE 6(b)

| Test No.         | Roll type | Shrinkage-fitting allowance |                | Stress A (kgf/mm <sup>2</sup> ) | Stress B (kgf/mm <sup>2</sup> ) | Rolling length until discarding ( $\times 10^3$ m) | Cause of discarding | Remarks                      |
|------------------|-----------|-----------------------------|----------------|---------------------------------|---------------------------------|----------------------------------------------------|---------------------|------------------------------|
|                  |           | $\sigma_{max}$              | $\sigma_{min}$ |                                 |                                 |                                                    |                     |                              |
| <u>Invention</u> |           |                             |                |                                 |                                 |                                                    |                     |                              |
| 1                | FIG. 14   | 0.160                       | 0.080          | 8                               | 16                              | 150-300                                            | Crack               | Favorable working efficiency |
| 2                | FIG. 14   | 0.160                       | 0.080          | 8                               | 16                              | 500 or more                                        | —                   | Favorable working efficiency |
| 3                | FIG. 14   | 0.160                       | 0.080          | 8                               | 16                              | 300-400                                            | Wear                | Favorable working efficiency |
| 4                | FIG. 14   | 0.160                       | 0.080          | 8                               | 16                              | 500 or more                                        | —                   | Favorable working efficiency |
| 5                | FIG. 14   | 0.160                       | 0.080          | 8                               | 16                              | 150-300                                            | Crack               | Favorable working efficiency |
| 6                | FIG. 14   | 0.160                       | 0.080          | 8                               | 16                              | 500 or more                                        | —                   | Favorable working efficiency |
| 7                | FIG. 14   | 0.160                       | 0.080          | 8                               | 16                              | 300-400                                            | Wear                | Favorable working efficiency |
| 8                | FIG. 14   | 0.160                       | 0.080          | 8                               | 16                              | 500 or more                                        | —                   | Favorable working efficiency |

In Table 6, stress A and stress B respectively denote the compressive stress caused by the recess gap of each roll, and the compressive stress caused by shrinkage-fitting, and the maximum tensile stress occurring during rolling is constant at 81 kgf/mm<sup>2</sup>. In all caliber rolls for rolling presented for the rolling process, an excellent resistance to wear and cracking is confirmed.

As this invention may be embodied in several forms without departing from the spirit of essential characteristics thereof, the present embodiment is therefore illustrative and not restrictive, since the scope of the invention is defined by the appended claims rather than by the description preceding them, and all changes that fall within the meets and bounds of the claims, or equiva-

lence of such meets and bounds thereof are therefore intended to be embraced by the claims.

What is claimed is:

1. A method of manufacturing a caliber roll for rolling comprising steps of:

inserting a roll shaft into a shaft hole of a roll main body, the roll main body having a caliber on an outer circumference thereof and the shaft hole penetrating therein in an axial direction; and applying a compressive stress in a widthwise direction of said roll main body to a bottom of the caliber, the compressive stress being applied by forming first and second spaced-apart tapered sections either on an internal circumference of the shaft hole of said roll main body or on a circumference of said roll shaft and shrinkage-fitting or cold-fitting said roll main body and said roll shaft, the first and second tapered sections being formed so as to provide a shrinkage-fitting or cold-fitting allowance which gradually decreases from opposed end faces of the roll main body towards a central part of the roll main body, and the first and second tapered sections on the internal circumference of the roll main body having diameters which both increase as the tapered sections become closer and closer together in the axial direction or the first and second tapered sections on the circumference of the roll shaft having diameters which both de-

30

crease as the tapered sections become closer and closer together in the axial direction.

2. The method of claim 1, further comprising: forming a recess gap in a middle of the internal circumference of the shaft hole of said roll main body

5 3. The method of claim 1, wherein the first and second tapered sections are formed on the roll shaft and comprise portions of the roll shaft which decrease in diameter towards the central part of the roll main body.

10 4. The method of claim 3, wherein prior to the inserting step the shaft hole is formed so as to have a uniform diameter between opposed end faces of the roll main body.

5 5. The method of claim 1, wherein the first and second tapered sections are portions of the shaft hole which increase in diameter toward the central part of the roll main body.

10 6. The method of claim 5, wherein prior to the inserting step the roll shaft is formed so as to have a uniform diameter between opposed end faces of the roll main body.

20 7. The method of claim 1, wherein the roll main body is formed by rolling or forging a billet such that the billet is rolled or forged in the axial direction.

25 8. The method of claim 1, wherein the roll main body comprises a single piece of material.

9. The method of claim 1, wherein the shaft hole and the caliber of the roll main body are surfaces of a single piece of material.

\* \* \* \* \*

35

40

45

50

55

60

65